

## COMBUSTIBLE COMPOSITION

David E. Pearsall, Avon, Conn., assignor to Bickford Research Laboratories Inc., Hartford, Conn., a corporation of Connecticut

No Drawing. Application February 8, 1957  
Serial No. 638,925

5 Claims. (Cl. 52—2)

The present invention relates generally to combustible or burning type compositions. More particularly it relates to compositions of this type which are oxygen-sufficient and which may be used in places in which black powder and other gaseous or thermit type powders have been used in the past, for example, in safety or blasting fuses, military fuses, delay elements for blasting caps, tracer and flare charges, igniting cord for the transmission of flame or fire from one point to another, fireworks and the like. By "oxygen-sufficient" is meant that the compositions of the present invention burn without the addition of any atmospheric oxygen.

Black powder, which is a mixture of charcoal, sodium or potassium nitrate and sulphur, has been used for many years as the burning composition in fuses and the like. Although satisfactory for many purposes, black powder has an inherent disadvantage which relates to the charcoal ingredient, i.e. it is variable in its nature and therefore the entire black powder composition is correspondingly variable in its characteristics and not always predictable as to rate of burning, the volume of gaseous products evolved, the temperature of combustion, etc. Since it is essential in certain of the uses above enumerated that the rate of burning and/or the amount of gas evolved shall be definitely predictable and determinate, black powder has therefore proved inadequate in supplying the needs of the art. In addition, black powder is susceptible to the humidity of its surroundings, readily taking up moisture with a consequent impairment of its efficiency. Also, black powder has a tendency to change on aging in certain characteristics, such as burning rate.

A principal object of the present invention is to provide a burning composition which may be used in general as a substitute for black powder and/or for other uses hereinabove enumerated and which may be relatively unaffected by the various conditions which deleteriously affect black powder such, for example, as humidity and aging and which shall be predictable in its characteristics within relatively narrow limits. The compositions of the present invention are readily duplicable, which is a characteristic not shared by black powder.

It is noted in this connection that the charcoal ingredient in black powder is made by the carbonization of wood, which is a highly variable natural occurring product. There are many different conditions of carbonization and many kinds of wood; wood from different portions of the same tree may have essentially diverse characteristics when made into charcoal. In addition to this, the charcoal made from naturally occurring wood is highly porous and hence subject to being affected by humidity conditions; it is often more or less adsorptive and hence is subject to variation by reason of the different amounts of different types of gases which may be adsorbed on the surface of the charcoal particles. By contrast to this, the compositions of the present invention utilize a uniform and substantially non-adsorptive

or inactive surface form of carbon as hereinafter more particularly set forth, so that the present compositions are uniform in their characteristics in use.

A further principal object of the present invention is to provide combustible or burning compositions in which the burning time may be adjusted within reasonable limits by adjustment of the proportions of various essential ingredients of the compositions; and more particularly in which the amount of gaseous products evolved upon burning may be varied and controlled within reasonable limits, exclusive of the burning time. So far as is known, the compositions of the present invention are the first ones wherein this dual adjustment of burning time and the proportionate amounts of gaseous products of combustion are independently adjustable.

Summarizing the present invention, it comprises a composition including as oxidizing agents (1) a non-gas-producing alkaline earth peroxide ( $BaO_2$ ) which is present to the extent of about 65% to 90%, and (2) a gas-producing alkali metal nitrate ( $KNO_3$ ) which is present to the extent of about 4% to 25%; and as fuels a non-gas-producing material such as metallic silicon which is present to the extent of about 1% to 10%, and a gas-producing material consisting of one or more particular types of carbon blacks present to the extent of about 1 to 15%. In addition to this, in some of the more highly refined embodiments of the invention, there may be added a binder which is a combustible organic plastic material, such as nitrocellulose and which is present to the extent of about 3% to 10% of the entire composition. Furthermore, in a particular preferred composition there may be added a desensitizing material comprising a metallic stearate, such as aluminum or zinc stearate, which may be present to the extent of about 0.1% to about 1.0%. It is within the intended scope of this invention that minor amounts of other ingredients may be added to improve the compositions in various minor respects.

The materials aforesaid, with the exception of the organic plastic binder, are preferably dry-mixed and blended together and then admixed with a volatile solvent-solution of the organic plastic binder (lacquer) to form a slurry, which may then be cast into thin sheets. After the solvent has evaporated therefrom, the cakes are broken down, grained, sieved to select a desired particle size, and the particles coated with graphite to improve their moisture-resistance and flow characteristics.

The details of the present invention will appear hereinafter from a particular discussion of the several ingredients, their characteristics and their equivalents, and also a discussion of the effects to be attained by varying the proportions of different ingredients.

Considering now the characteristics of the several essential ingredients, there are in this composition, as in most mechanical mixture types of burning compositions, one or more oxidizing agents and one or more fuels. In this case there is a non-gas-producing and a gas-producing oxidizer and a non-gas-producing and a gas-producing reducer or fuel.

In the class of oxidizing agents, the first element which is present to the extent of 65% to 90% of the weight of the active ingredients of the composition is a low gas producing alkaline earth peroxide such as barium peroxide ( $BaO_2$ ). The weight proportions given in the examples hereinafter given apply particularly to barium peroxide.

As a non-gas-producing fuel, the present invention utilizes metallic silicon.

It is recognized that if barium peroxide and silicon were mixed, with no other materials present, a non-gas-producing burning composition of the thermit type would be provided. It is believed, however, that such a com-

position would not fulfill all the requirements in the present case, as it would not provide for the evolution of any gas, some of which is needed, for example, in connection with fuse powders to provide an "end-split," that is, an evolution of highly heated gaseous products of combustion and/or sparks or flames as required to ignite a charge at the termination of the burning of a length of fuse.

According to the present invention there is also provided a high oxygen producing alkali metal nitrate, such as potassium nitrate. This material, when reacted, furnishes a readily available supply of oxygen and provides additional gaseous products such as nitrogen or some oxide thereof.

In addition, there is present according to the invention a gas-producing type of fuel, namely carbon black, but only in one or more of certain selected and particular types. Carbon black usable in the present compositions may be generally of three groups consisting of (a) furnace black and thermal furnace blacks, (b) acetylene blacks and (c) synthetic graphites. Processes for making the various forms of carbon aforesaid are described in the book "Industrial Carbon" by C. L. Mantell (published by D. Van Nostrand Company, Inc., of New York city in 1946).

The preferred carbon blacks, known as furnace and thermal furnace blacks, respectively, are those characterized by having low adsorptive capacity or surface activity. Channel blacks are not acceptable according to the present invention.

Satisfactory forms of carbon or blacks for the purposes of this invention have properties as listed below:

|                                     |                         |
|-------------------------------------|-------------------------|
| Average particle size               | 40 to 500 millimicrons. |
| Fixed carbon content                | 98% (minimum).          |
| Volatile content                    | 2% (maximum).           |
| Hydrogen ion values                 |                         |
| Diphenyl guanidine adsorption value | 7-11.                   |
| Oil adsorption value                | 10 (maximum).           |
|                                     | 40 to 90.               |

These values are obtained by methods familiar to the carbon and pigment industries and described in the book above referred to.

If the composition were made up, for example, with nothing but barium peroxide and silicon, there would be little or no gas evolution on burning; whereas if the composition were solely potassium nitrate and carbon, there would be considerable gaseous evolution upon burning. The preferred compositions are somewhere between these two extremes and in practice are such that the products of combustion will be about 10% to 18% (by weight) gaseous and the balance solid. The higher limits of this range of variation are attained by proportionately increasing the content of the gas-producing ingredients and correspondingly reducing the proportions of non-gas-producing ingredients, both as above defined.

The next variable to be particularly considered is the speed of burning. This is important when the composition is to be used in the making of safety fuse, for example, where fuses are required to burn at definite rates. As previously set out, it is possible to control the burning rate of the compositions of the present invention by proper adjustment of the proportions of the several ingredients. This proportioning is effected in view of the following principles: The barium peroxide is usually held fairly constant and the other three materials varied. It is possible, however, to make different burning rate powders over a fairly wide range of barium peroxide content, thus varying the amount of gas produced. When the proportions of carbon and silicon are

relatively high, the speed of combustion is relatively faster; when these fuels are reduced, the speed of combustion is slowed. Replacing a part of the silicon with carbon increases the amount of gas and vice versa. As to the nitrate, increased proportions of this ingredient result in progressively slower burning rates and higher amounts of gas and vice versa.

Another possible control of burning rate is in the particle size of the carbon used, finer particles of carbon in general producing faster burning power. When graphite is used as the carbon ingredient, a slower burning powder is produced than with other types of carbon black which are usable in accordance with the definition given above. Thus, a further way to provide a relatively slower burning powder is to replace a certain amount of the carbon black with graphite.

Another way to control the speed of burning of compositions according to this invention is to select a type of carbon within the limits above given, but with different adsorptive characteristics, those types having higher adsorption characteristics, as measured by higher diphenyl guanidine values, producing faster burning powders.

In general, the powders or compositions according to the present invention provide relatively less gas evolution per unit of weight than a corresponding weight of black powder. The calorific values of the burning compositions of the present invention may be relatively lower than those of black powder, but they usually burn at higher temperatures, which is very desirable for certain uses.

For ease in handling and use, it is desired that the compositions, which are basically in accordance with the present invention, shall be fabricated in a form of a grained powder. In order to produce a commercially usable powder in grained form, it is desired to mix the powder ingredients in finely divided form (100 mesh and smaller) with a binder material which comprises a combustible organic plastic insoluble in water, but soluble in conventional aliphatic organic solvents i.e. 40 a lacquer. The preferred binder in accordance with the present invention is a nitrocellulose (soluble in esters and ketones) having a nitrogen content of about 12% and a viscosity in the range of about 60 to 175 seconds. If it be considered that the four essential ingredients 45 shall be present in the proportions aforesaid so as to make up collectively 100 parts by weight, then there should be added from about 3 to about 10 parts by weight of nitrocellulose in the form of a lacquer. Once the nitrocellulose lacquer slurry is dried, the process 50 of making the powder as described above is substantially the same as known processes of preparing grained black powders. The process of this invention, however, effectively eliminates the cumbersome wheel mills and presses 55 which have been conventionally used in black powder manufacture and at the same time produces a combustible material having a high density by reason of the effective displacement by the liquid binder of air from the interstices between the particles making up the composition, followed by careful vaporization of the solvent 60 so as to leave the cake in substantially unchanged condition.

In some instances it may be desired to use additional ingredients in the composition prior to the making up 65 of the slurry as aforesaid, these ingredients being, for instance, for decreasing the moisture and water susceptibility of the composition, decreasing the sensitivity of the composition to impact, friction or spark or, perhaps, raising the ignition temperature of the composition. 70 Such an added material may be a metallic stearate, such as aluminum stearate and zinc stearate, and may be present in the final composition in an amount varying from about 0.1 to 1.0 part by weight based upon 100 such parts for the four essential ingredients as aforesaid. The compositions of the present invention may be

further illustrated by examples of compositions embodying this invention as follows:

*Example 1*

The active ranges of ingredients of preferred compositions according to the present invention may be listed as follows:

|                                  | Percent |
|----------------------------------|---------|
| Barium peroxide                  | 65-90   |
| Potassium nitrate                | 4-25    |
| Silicon                          | 1-10    |
| Carbon black (as herein defined) | 1-15    |

*Example 2*

Examples of relatively slow burning powders consisting essentially of the four active ingredients above defined are in the following ranges:

| Ingredient:           | Compositions, percent |
|-----------------------|-----------------------|
| BaO <sub>2</sub>      | 70-87                 |
| KNO <sub>3</sub>      | 6-20                  |
| Si                    | 2-6                   |
| C (as herein defined) | 1-4                   |

*Example 3*

Compositions having medium burning rates would be found in the following ranges of ingredients:

| Ingredient:           | Compositions, percent |
|-----------------------|-----------------------|
| BaO <sub>2</sub>      | 70-86                 |
| KNO <sub>3</sub>      | 5-21                  |
| Si                    | 3-6                   |
| C (as herein defined) | 3-6                   |

*Example 4*

Compositions having relatively fast burning rates are as follows:

| Ingredient:           | Compositions, percent |
|-----------------------|-----------------------|
| BaO <sub>2</sub>      | 70-85                 |
| KNO <sub>3</sub>      | 4-15                  |
| Si                    | 4-6                   |
| C (as herein defined) | 5-13                  |

*Example 5*

An example of a grained powder, including not only the four essential ingredients hereinabove given, but also the nitrocellulose binder and aluminum stearate, and which may be considered as one of the preferred embodiments of the invention is as follows:

|                            | Percent |
|----------------------------|---------|
| Barium peroxide            | 79.5    |
| Potassium nitrate          | 5.6     |
| Silicon                    | 5.6     |
| Carbon (as herein defined) | 2.8     |
| Nitrocellulose             | 6.0     |
| Aluminum stearate          | 0.5     |

In the foregoing disclosure there are set out the essential ingredients of compositions according to the present invention, the proportions in which these ingredients may be present in the composition as a whole, and the effects of changing the proportions within the limits given to attain certain specific and desired results.

It is intended that the scope of this invention shall be measured by the appended claims, which are to be construed validly as broadly as the state of the prior art permits.

What is claimed is:

1. An oxygen-sufficient combustible composition for use in safety fuses and the like and which provides independent adjustability of the burning time and of the amount of gases evolved, said composition comprising the following ingredients in the weight proportion stated:

|                     | Percent |
|---------------------|---------|
| BaO <sub>2</sub>    | 65-90   |
| KNO <sub>3</sub>    | 4-25    |
| Si                  | 1-10    |
| Carbon (as defined) | 1-15    |

all said ingredients being present in a particle size of not larger than about 100 (Tyler) mesh; said carbon being selected from the group consisting of (a) furnace blacks and thermal furnace blacks, (b) acetylene blacks and (c) synthetic graphites, said carbon further having the following properties:

|                                     |                         |
|-------------------------------------|-------------------------|
| Average particles size              | 40 to 500 millimicrons. |
| Fixed carbon content                | 98% (minimum).          |
| Volatile content                    | 2% (maximum).           |
| Hydrogen ion values                 | 7-11.                   |
| Diphenyl guanidine adsorption value | 10 (maximum).           |
| Oil adsorption value                | 40 to 90.               |

2. An oxygen-sufficient combustible composition in accordance with claim 1, comprising in addition a metallic stearate selected from the group consisting of aluminum and zinc stearates and serving as a desensitizer and present in an amount of about 0.1 to about 1.0 part by weight per 100 parts of the total materials recited in claim 1.

3. An oxygen-sufficient combustible composition in accordance with claim 1, comprising in addition a binder which is present in an amount of about 3% to about 10% by weight per 100 parts by weight of the total of materials recited in claim 1.

4. An oxygen-sufficient combustible composition in accordance with claim 1, comprising in addition nitrocellulose serving as a binder which is present in an amount of about 3% to about 10% by weight per 100 parts by weight of the total of materials recited in claim 1.

5. An oxygen-sufficient combustible composition in accordance with claim 1, which is present in the form of a grained powder and which consists essentially of the following ingredients (by weight):

|                       | Percent |
|-----------------------|---------|
| Barium peroxide       | 79.5    |
| Potassium nitrate     | 5.6     |
| Silicon               | 5.6     |
| Carbon (as aforesaid) | 2.8     |
| Nitrocellulose        | 6.0     |
| Aluminum stearate     | 0.5     |

References Cited in the file of this patent

UNITED STATES PATENTS

|           |          |               |
|-----------|----------|---------------|
| 1,415,889 | Mardick  | May 16, 1922  |
| 1,709,498 | Sorensen | Apr. 16, 1929 |
| 1,971,502 | Piccard  | Aug. 28, 1934 |
| 2,416,639 | Pearsall | Feb. 25, 1947 |
| 2,497,387 | Zenftman | Feb. 14, 1950 |
| 2,590,060 | Zenftman | Mar. 18, 1952 |

FOREIGN PATENTS

|    |        |               |      |
|----|--------|---------------|------|
| 65 | 26,617 | Great Britain | 1901 |
|----|--------|---------------|------|

UNITED STATES PATENT OFFICE  
CERTIFICATE OF CORRECTION

Patent No. 2,909,418

October 20, 1959

David E. Pearsall

It is hereby certified that error appears in the printed specification of the above numbered patent requiring correction and that the said Letters Patent should read as corrected below.

Column 3, line 11, before "potassium" insert -- as --; lines 39 and 40 should appear as shown below instead of as in the patent:

-- Hydrogen ion values \_\_\_\_\_ 7-11.  
Diphenyl guanidine adsorption \_\_\_\_\_ --;

column 4, line 4, for "vice versa" read -- vice versa --; line 10, for "power" read -- powder --; column 6, line 19, "particles" read -- particle --.

Signed and sealed this 3rd day of May 1960.

(SEAL)  
Attest:

KARL H. AXLINE  
Attesting Officer

ROBERT C. WATSON  
Commissioner of Patents